

## UNITED STATES PATENT OFFICE.

ARTHUR M. HOWALD, OF PITTSBURGH, PENNSYLVANIA, ASSIGNOR TO THE GRASSELLI CHEMICAL COMPANY, OF CLEVELAND, OHIO, A CORPORATION OF OHIO.

## WOOD IMPREGNATION.

No Drawing.

Application filed November 30, 1926. Serial No. 151,838.

This invention relates to the preservation of wood by the impregnation thereof with oily wood preserving agents. More particularly, it relates to the treatment of oily wood-  
5 impregnating materials or mixtures for the purpose of improving their penetrative powers thus shortening and making more easy the process of impregnating wood with same.

As is well known, wood is preserved by im-  
10 pregnating same with petroleum oils, coal tar oils, wood tar oils, mixtures of these, and the like. In the preservation of wood with these oily agents a thorough penetration is desired for which purpose seasoning or drying of the  
15 wood, steaming of the wood, and during the impregnation, vacuum, pressure, and high temperatures are resorted to.

The present invention relates to the treatment of impregnating oils whereby they are  
20 rendered more penetrative and the ease of injecting them into wood for thorough penetration is thereby greatly increased.

It has been found that if oily wood impregnating agents, regardless of their viscosity, be  
25 treated with acids, their ease of injection into wood is materially increased and the time, pressure, and temperature required to obtain a given impregnation may be correspondingly decreased. Also if the usual conditions of  
30 treatment are adhered to a greater depth and completeness of penetration and corresponding preservative effect may be obtained.

In practicing this invention the oily impregnating agent, preferably warmed, is agi-  
35 tated with the acid (a 30 per cent solution or other convenient strength of sulfuric acid may be used), after which the mixture is al-  
lowed to stand, the acid settles out, and may be used for treating additional quantities of  
40 impregnating oil.

Any convenient strength of sulfuric, hydrochloric, phosphoric or other acid, or acid salt such as niter cake, waste acids from petroleum refining, etc., may be used. A con-  
45 venient method of practicing this invention is to add to the hot impregnating oil 5 per cent of a 30 per cent solution of sulfuric acid, agitate vigorously with air, allow to settle and draw off the acid solution whereupon the  
50 oil may be used for wood impregnation with improved results.

Effects amounting to an increase of from 100 to 500 per cent in the amount of oil in-  
55 jected into the wood under otherwise equal conditions have been obtained. A 50-50

mixture of creosote oil and petroleum resi-  
duum (a viscous residue of petroleum usu-  
ally used as fuel) treated by the procedure  
described, i. e., washed with sulfuric or other  
acid of any convenient strength, for instance,  
60 30 per cent sulfuric acid, in almost any quan-  
tity, say 0.5 to 5 per cent by volume and up-  
wards, can be made to completely impregnate  
wood in a much shorter time and at a lower  
65 pressure than the untreated mixture.

As has been indicated the treatment of the oily impregnating agent is applicable to such agents generally and is not limited to any particular acid or strength or quantity thereof but the acid preferably is used in  
70 quantity and concentration insufficient to effect refining of the oil or oily impregnating agent.

No definite theory explaining the effect of the acid treatment upon the oily impregnating agent has been determined. The change in the oil as a result of the acid treatment evi-  
dently results in a change in the capillarity  
relations of the oil and the wood whereby the  
oil more readily wets the wood and is more  
80 easily forced into its minute pores. Al-  
though it appears that the change in the acid-  
ity of the oil produces the change in its pene-  
tration properties since washing the oil with  
alkali has an opposite effect, it has been ob-  
85 served that no more than a negligible quan-  
tity of acid or alkali is retained by the treated  
oil in either case. The invention is particu-  
larly valuable in the treatment of woods  
90 which are difficult to impregnate with oily preservative materials, such as fir, spruce,  
and the like.

The acid treatment of oily wood impregnating agents for the purpose of improving their penetrative properties in accordance with the invention is to be clearly distin-  
95 guished from the refining of oils, particularly petroleum oils, by acid treatment. The acid treatment ordinarily used for refining oils, for instance the typical treatment with  
100 sulfuric acid of about 60° Bé., is not applica-  
ble for improving the penetrative properties of wood preserving oils in accordance with the invention and oils which are ordinarily refined by the 60° Bé. sulfuric acid treat-  
105 ment are not ordinarily considered as wood preserving oils and the effects of the acid treatments of the two types of oils are different. The refining of mineral oils by means of acid ordinarily requires concen-  
110

trated acid, i. e., 60° Bé. sulfuric acid which reacts with certain unstable and reactive constituents of the oil and results in a clarification of the oil and improvement in its odor and ageing properties, whereas the acid treatment of the invention requires only weak acid of say up to 30° Bé. sulfuric acid which does not appreciably react with the unstable and reactive constituents of the oil and does not clarify or deodorize it or improve its ageing properties, i. e., it does not exert an appreciable refining effect. Mineral oils which are customarily refined by means of sulfuric acid of about 60° Bé. contain only a relatively small amount of unstable and reactive constituents whereas wood preserving oils ordinarily contain a relatively large proportion of unstable and reactive constituents. These unstable and reactive constituents in wood preserving oils would be removed by strong acid treatment which would involve a prohibitive consumption of acid and would leave only a relatively small amount of refined oil which would not be desirable for wood preserving purposes. Thus the acid treatments for refining oils and for improving their penetrative properties in accordance with the invention are different, particularly with respect to the kind and concentration of acid used, the oils treated are different, and the desired results and the results actually obtained are different.

I claim:

1. Process of improving the penetrative properties of oily wood impregnating agents, which comprises contacting an oily wood impregnating agent with an acid of a concentration and in quantity insufficient to effect refining of the oily wood impregnating agent.
2. Process of improving the penetrative properties of oily wood impregnating agents, which comprises contacting an oily wood im-

pregnating agent with a solution of a strong mineral acid of a concentration and in quantity insufficient to effect refining of the oily wood impregnating agent.

3. Process of improving the penetrative properties of oily wood impregnating agents, which comprises contacting an oily wood impregnating agent with about 5 per cent by volume of a solution of a mineral acid in a concentration insufficient to effect refining of the oily wood impregnating agent.

4. Process of improving the penetrative properties of oily wood impregnating agents, which comprises contacting the oily wood impregnating agent with about 5 per cent by volume of a 30 per cent solution of sulfuric acid.

5. Process of improving the penetrative properties of oily wood impregnating agents, which comprises agitating the oily wood impregnating agent with a relatively small proportion of a dilute solution of a strong mineral acid, and separating the acid solution from the oily material.

6. Oily wood impregnating agents obtainable by washing oily wood preserving materials with acids of a concentration and in quantity insufficient to effect refining of the oily wood preserving materials, said agents retaining only negligible quantities of said acids and having penetrative properties at least 100% greater than the corresponding untreated materials.

7. An oil wood impregnating agent resulting from the treatment of an oily material capable of use for wood impregnation with a relatively small quantity of a comparatively dilute solution of a strong mineral acid, said agent having penetrative properties at least 100% greater than those of said oily material.

In testimony whereof, I affix my signature.

ARTHUR M. HOWALD.